

## UNITED STATES PATENT OFFICE

RUSSELL L. BROWN, OF LOWELL, MASSACHUSETTS, ASSIGNOR, BY MESNE ASSIGNMENTS,  
TO FITGER CALIFORNIA COMPANY, OF LOS ANGELES, CALIFORNIA, A CORPORATION  
OF CALIFORNIA

## PROCESS OF CLEANING WOOL AND OTHER ALLIED FIBERS

No Drawing.

Application filed September 15, 1932. Serial No. 633,378.

Fleece wool as it is sheared from live sheep, and pulled wool, as it is pulled from the skins from slaughtered sheep, and allied fibers, such as the hair of the camel, mohair, llama 5 hair, alpaca, and goat hair, all contain fiber which is keratin, suint (the salts of perspiration) and grease, or yolk (degras), and foreign matter which consists of sand, dirt, dust, vegetable matter of various kinds and hy- 10 groscopic moisture.

This invention is a process of removing from the fleece or pulled wool or other allied fibers a portion of the degras (yolk) or grease, and all or a substantial portion of the foreign 15 matter such as sand, dirt, dust, vegetable matter and the like adhering thereto.

I have discovered that so-called "fleece wool", or "pulled wool" or other allied fibers can be cleaned of foreign matters and a portion 20 of the grease (yolk or degras) etc. adhering thereto without any moistening or other preliminary treatment by subjecting it to a temperature sufficiently low to stiffen or congeal the grease or degras on the fiber and 25 foreign matters but not freeze the fibers, and then removing a portion of the grease and substantially all of the foreign matters by passing the refrigerated fibers through a mechanical device, such as a so-called dusting 30 or picking machine, whereby a portion of the cold grease and practically all of the foreign matters are separated from the fibers, the latter being discharged from the mechanical device substantially cleaned of burrs, chaff, and 35 other vegetable matter, sand, and dirt, and an appreciable portion of the grease.

Natural untreated fleece or pulled wool and/or other allied fibers contain more or less natural grease, and such grease more or 40 less coats the burrs, vegetable and foreign matters, and if such wool or fibers are subjected to a temperature sufficient to harden or congeal the grease it renders the burrs, vegetable and foreign matters sufficiently 45 solid to enable them to be readily detached from the fibers. There may be a natural wax in the vegetable matter which further assists in making it more susceptible to removal at refrigerated temperatures.

50 In carrying out my invention the fleece or

pulled wool or other allied fibers are assorted in the usual manner, and when it is desired to clean the same, the fleece or pulled wool or other fibers, without any preliminary washing or moistening, may be placed in a feeder 55 and preferably fed into or onto a conveyor, preferably an endless belt, whereon the wool or fibers are chilled to a temperature sufficient to stiffen or congeal the grease, either by having the conveyor confined in a chamber at a refrigerated temperature, or by subjecting the wool or other fibers to refrigerated air. As the grease will harden or congeal very 60 quickly the time required for this chilling is short.

The chilled wool or other fibers are then 65 fed into a so-called "duster" or cleaning machine whereby the congealed grease and foreign matters are detached from the wool or other fibers.

In actual tests I have found very substantial cleaning can be effected at temperatures as high as 35° F. and as low as minus 15° F., but I do not restrict myself to this range of 70 temperatures. The time of chilling may vary from less than one minute to about ten minutes or more, depending upon the nature of the wool or other fibers and upon the temperature. The grease should be chilled sufficiently to render it hard enough to hold the 75 vegetable matter intact. In the fleece or unwashed state the burrs and foreign matters are not so matted in or with the wool or other fibers as they are if the wool or other fibers are scoured and/or washed before they are 80 refrigerated, and therefore the foreign matters can be more readily detached.

85 After the separation of the foreign matters from the wool or other fibers, the wool or other fibers may be placed in storage or 90 shipped without any further treatment, or may be passed through the usual scouring bowls, or degreasing machines, or washing machines, and then dried or passed into the manufacturing plant for use. The scouring, 95 decreasing and/or washing would be done more rapidly, with less detergents, and with less expense than is necessary by present methods.

In my invention it is not necessary or de- 100

sirable to moisten or wash or degrease the wool or other fibers prior to the cleansing operation; and I dispense with the initial dusting or opening and cleansing and washing steps, or the wetting heretofore used, prior to the refrigerating and the separating steps, and this leaves the wool or other fibers in a condition more desirable for subsequent operations. In tests of my process I have taken the fleece, pulled wool, or other fibers, and dried same in an oven, even to a bone-dry state, and then treated same by my process with the result that much of the grease and substantially all of the foreign matters were removed.

By not moistening or washing the wool or other allied fibers prior to refrigeration, I obviate the necessity for careful control of the moisture content before freezing, and the use of excess water in the fibers, which excess water prolongs the time and increases the expense of refrigeration. I have found that the mestiza (spiral or watch-spring) burr becomes very weak and flattened if/when passed through the scouring operation and squeeze rolls, and has a tendency to unwind. Since I treat the wool or other fibers prior to scouring, the burrs retain their natural shape and strength when introduced into my process. The absence of water other than hygroscopic moisture in my process, results in less corrosion of the machinery, and less expense in removing frozen moisture discharged from the dusting machine. Also it is possible to use my invention without the expense of drying equipment, and the product can be stored or shipped without further treatment, which can not be done by the wet refrigeration process. By my process the wool or other allied fibers have substantially all the foreign matters, and considerable of the grease, removed before it is degreased, washed, or scoured; therefore less detergents are required for cleansing than by other known processes. The burrs also are much easier to remove because they have not been previously water-soaked and flattened by passing through the squeeze rolls before separation, as has been heretofore customary.

The equipment necessary to carry out my process is simple and can be more readily installed in existing plants than the wet freezing process, because much less refrigeration is required, and it can be located any place in the plant rather than after the scouring apparatus as required by the wet freezing process.

I claim:—

1. The herein described process of cleaning unwashed fleece and pulled wools and other allied animal fibers, containing extraneous foreign matters and substantially all the natural grease as derived from the animal, consisting in subjecting such wools and other

allied fibers to a low temperature which will congeal the grease on the wools or fibers, and then cleaning the wools or fibers by mechanical means while at the low temperature.

2. The herein described process of cleaning unwashed fleece and pulled wools and other allied animal fibers containing extraneous foreign matters and substantially all the natural grease as derived from the animal, of foreign matters, consisting in subjecting such wools or other allied fibers to a low temperature which will congeal the grease on the foreign matters, and while congealed substantially removing the foreign matters by mechanical means.

3. The herein described process of cleaning unwashed fleece and pulled wools and other allied animal fibers containing extraneous foreign matters and substantially all the natural grease as derived from the animal, of foreign matters and a portion of the grease, consisting of subjecting such wools or other allied fibers to a low temperature which will congeal the grease on the foreign matters and wools or fibers, and while congealed removing the foreign matters and a portion of the grease from the wools or fibers by mechanical means.

4. The herein described process of cleaning fleece and pulled wools and other allied animal fibers of foreign matters and a portion of the grease adhering to the wools or fibers as derived from the animal prior to washing or scouring the wools or fibers, consisting in subjecting such wools or other allied fibers to a low temperature which will congeal the grease on the wools or fibers and foreign matters, and then while congealed detaching the foreign matters and a portion of the grease from the wools or fibers by mechanical means.

5. The herein described process of cleaning unscoured fleece and pulled wools and other allied animal fibers, containing extraneous foreign matters and substantially all the natural grease as derived from the animal, of foreign matters; consisting in subjecting such wools or other allied fibers to a low temperature which will congeal the grease on the foreign matters, and while congealed separating the foreign matters by mechanical means.

RUSSELL L. BROWN.

120

125

130